

# United States Patent Office

2,895,914

Patented July 21, 1959

1

2,895,914

## PROCESS OF FORMING NAPHTHENIC ACID SOLUTIONS

Rudolf Kern, Neustadt, Hans Scheurer, Heidelberg, Hermann Zorn, Mannheim, and Eugen Kruppke, Heidelberg, Germany, assignors to Firma Rhein-Chemie G.m.b.H., Heidelberg, Germany

No Drawing. Application April 3, 1953  
Serial No. 346,784

Claims priority, application Germany April 12, 1952

27 Claims. (Cl. 252—37)

The present invention relates to naphthenic acid solutions and processes of making the same and more particularly to liquid hydrocarbon solutions of naphthenic acid salts which are especially suitable for motor oils and lubricating oils.

Naphthenic acid salts have been utilized in mixture with organic solvents and particularly hydrocarbons in various chemical fields, especially for the manufacture of impregnating agents, pesticides, plastics, etc.

Naphthenic acid salts have also been added to motor oils and lubricating oils in order that the cation of the naphthenic acid salt might react with and neutralize the free sulfuric acid which is formed upon burning of the sulfur-containing oil. Mainly polyvalent metal salts of naphthenic acid were utilized for this purpose, i.e. barium and aluminum naphthenates. However, the use of these naphthenic acid salts was greatly limited and made extremely difficult because of the physical characteristics of the same, particularly when mixed with liquid hydrocarbons.

The naphthenic acid salts are either insoluble or only difficultly soluble in hydrocarbons, or the naphthenates form gels with the hydrocarbons. The naphthenic acid salts therefore greatly increase the viscosity of the hydrocarbons to which they are added. This increase in viscosity is highly detrimental for many purposes and therefore prevents the use of the naphthenic acid salts and particularly the polyvalent metal salts of naphthenic acid for such purposes.

It has been attempted to overcome these drawbacks in the use of naphthenic acid salts by the addition thereto of many different substances. However until the present time none of these additions have proved successful and the difficult solubility of the naphthenic acid salts and the high viscosities of the solutions of the naphthenic acid salts in hydrocarbons has proved to be an important problem in many industries.

It is therefore an object of the present invention to provide means for dissolving naphthenic acid salts in liquid hydrocarbons and hydrocarbon oils consisting of mixtures of hydrocarbons whereby greater quantities of the naphthenic acid salts can be dissolved in the liquid hydrocarbon without unduly increasing the viscosity of the hydrocarbon.

It is a further object of the present invention to provide for means of dissolving naphthenic acid salts in liquid hydrocarbons whereby the viscosity of the naphthenate-containing liquid hydrocarbon is much lower than the viscosity of the ordinary hydrocarbon solutions of naphthenic acid salts containing the same amount of naphthenate and whereby the resinification products and other decomposition products of the liquid hydrocarbon oils are dissolved or dispersed in the hydrocarbon.

It is a still further object of the present invention to provide for the formation of clear solutions of naphthenic acid salts in liquid hydrocarbons.

It is another object of the present invention to pro-

2

vide a group of compounds any member or members of which may be utilized as intermediates for the dissolution of naphthenic acid salts in liquid hydrocarbons.

It is still another object of the present invention to provide a second group of compounds which when utilized in addition to the first group of compounds further increases the dissolving ability of liquid hydrocarbons for naphthenic acid salts, the second group of compounds increasing the effect of the first group of compounds when utilized simultaneously therewith.

With the above objects in view, the present invention mainly comprises in a process of forming hydrocarbon and hydrocarbon oil solutions of naphthenic acid salts, the step of mixing a naphthenic acid salt with a liquid hydrocarbon and with at least one substance having the general formula:  $XO-(R-O)_n-R-OY$ , wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of the groups X and Y is selected from the class consisting of alkyl, aryl, aralkyl, alkaryl, alicyclic and acyl radicals having at least 6 carbon atoms.

The above group of compounds represented by the general formula  $XO-(R-O)_n-R-OY$  will hereinafter be referred for convenience as solvent A.

It has been found according to the present invention that solvent A increases the solubility of the naphthenic acid salts in the liquid hydrocarbons either by serving as intermediate solvent therefor or by some unknown action. The manner in which the solvent A works is unimportant, the present invention not being limited to any theory of operation but rather to the fact that solvent A does have the desired action.

In addition it has been found that the incorporation of a second group of substances having the general formula:  $R'-O-R''$  wherein R' and R'' are alkyl, aryl, aralkyl, alkaryl or alicyclic groups and at least one of the groups R' and R'' contains at least 6 carbon atoms further increases the dissolving ability of the liquid hydrocarbon for the naphthenic acid salts. This second group of substances will hereinafter be referred to as solvent B.

It should be noted that solvent B may be utilized in addition to solvent A and not in place of solvent A. Solvent A is absolutely necessary for the sufficient improvement in the dissolution of the naphthenic acid salts in the liquid hydrocarbons. Solvent B when used in addition to solvent A provides the advantage of forming clear solutions of the naphthenic acid salts.

The term "naphthenic acid salts" refers to any metal salt of naphthenic acid and particularly polyvalent metal salts of naphthenic acid. Aluminum naphthenate, barium naphthenate, calcium naphthenate, zinc naphthenate, iron naphthenate, lead naphthenate, potassium naphthenate, and the like naphthenates are examples of naphthenic acid salts which may have the solubility thereof in hydrocarbons increased according to the present invention, the scope of said invention now however being limited to the specific naphthenates mentioned.

As stated above, solvent A has the general formula:  $XO-(R-O)_n-R-OY$  wherein R is an alkylene radical of 2 or 3 carbon atoms, n is a whole number between 1 and 20 and either X or Y is a hydrogen, alkyl, aryl, aralkyl, alkaryl, alicyclic or acyl radical of any number of carbon atoms and the other of the groups X and Y is an alkyl, aryl, aralkyl, alkaryl, alicyclic or acyl radical of at least 6 carbon atoms.

It is preferred that n be between 2 and 7. It is further preferred that the radical X or Y which must be of at least 6 carbon atoms, be of at least 8 carbon atoms,

and still more preferably that it be exactly 12 carbon atoms. There is no actual maximum as to the number of carbon atoms for the groups X and Y, though as a practical matter X and/or Y should not have more than 24 carbon atoms.

In the above given general formula for solvent A, it may be seen that the portion: O—(R—O)<sub>n</sub>—R—O of the compound is symmetrical and therefore any radical which may be substituted for X may equally be substituted for Y. Thus, either or both X and/or Y may be substituted by an alkyl, aryl, aralkyl, alkaryl, alicyclic or an acyl group. Either X or Y, but not both, may be substituted by a hydrogen radical. If one of the groups X or Y is substituted by a hydrogen radical, then the other group must be substituted by an alkyl, aryl, aralkyl, alkaryl, alicyclic or an acyl radical of at least 6, preferably at least 8 and most preferably exactly 12 carbon atoms. If both groups X and Y are substituted by alkyl, aryl, aralkyl, alkaryl, alicyclic or acyl radicals, then only one of the groups must be of at least 6 carbon atoms, although both groups may be of at least 6 carbon atoms. The alkyl, aryl, aralkyl, alkaryl, alicyclic or acyl groups may be either saturated or unsaturated.

It is therefore apparent that solvent A is either an esterified or etherified polyalkylene glycol or esterified or etherified ester or ether derivative of polyalkylene glycol in which there are at least 2 and at most 21 alkylene groups and in which the polyalkylene glycol is esterified or etherified with at least one radical having at least 6 carbon atoms. The solvent A may be a monoether, a diether, a monoester, a diester, or an ether-ester of polyalkylene glycol. Preferably the solvent A will contain five alkylene groups and the alkyl, aryl, aralkyl, alkaryl, alicyclic or acyl group will contain 12 carbon atoms.

The following are examples of different compounds which may be utilized as solvent A according to the present invention. It is to be understood that these examples are given for illustrative purposes only and the scope of the present invention is in no way meant to be limited to the specific compounds mentioned.

The following are examples of monoethers of polyalkylene glycol:

Dodecylpentaethylene glycol, octadecenyl-hexaethylene glycol, laurylpentaethylene glycol, 2-ethylhexylpentaethylene glycol, nonylheptaethylene glycol, phenylethylpentaethylene glycol, methyl-cyclohexylctaethylene glycol, p-octylphenyltetrapropylene glycol, dodecylcyclohexyl-hexapropylene glycol, hexylnaphthyltetraethylene glycol and hexylnaphthyltetrapropylene glycol.

The following are examples of diethers of polyalkylene glycol:

Dodecyl- or laurylpentaethyleneglycolmethyl ether (the term lauryl should be understood as designating the radical from fatty alcohol produced from coconut fatty acids), p-octylphenyl-tetraethyleneglycolisopropylether, octydecenyl-hexaethyleneglycol-ethylhexyl ether, 2-ethylhexyl-heptaethylene glycolbenzylether, etc. It is to be noted that any alcohol may be utilized for the esterification of the polyalkylene glycol, including alcohols obtained by the reduction of natural or synthetic fatty acids, by the carbon monoxide hydrogenation at normal or raised pressure, by the oxo-synthesis or by paraffin oxidation.

The following are examples of mono and diesters of polyalkylene glycol and of ethers of polyalkylene glycol:

Pentaethyleneglycol-monostearate, hexaethylene-glycol-monostearate, dodecylbenzyl-pentapropylene glycol-oleate stearoyl-pentaethylene glycol-isopropylether stearoyl-pentapropylene glycol-isopropylether, benzoylpentaethylene-glycol-oleate, benzoylheptaethylene- or propylene-octylether, and benzoylpentaethyleneglycolmethyl ether.

The production of solutions of naphthenic acid salts in hydrocarbons according to the process of the present invention can be accomplished in various ways. The

method of proceeding depends upon the specific naphthenate, polyalkylene glycol derivative and the hydrocarbon oil in which the substances are mixed. It is preferable, although not necessary, to work at raised temperatures i.e. between 90-150° C.

The components, namely the naphthenate, polyalkylene glycol derivative and the hydrocarbon oil may be mixed together, preferably while stirring and at raised temperature, or the polyalkylene glycol derivative may be first mixed with the hydrocarbon and then the naphthenic acid salt added, or the naphthenic acid salt may be mixed with the hydrocarbon and the polyalkylene glycol derivative added, or the polyalkylene glycol derivative first mixed with the naphthenic acid salt and the thus formed solution then added to the liquid hydrocarbon.

The amount of solvent A, namely the polyalkylene glycol derivative, can be varied within very wide ranges, for example from 1% by weight of the amount of naphthenate to equal or even more than the amount of naphthenate. The specific amount depends upon the type of naphthenate as well as upon the use to which the hydrocarbon solution of the naphthenate is to be put and on the desired viscosity of the final solution. Anyone skilled in the art can by simple pretesting determine the exact amount of solvent A to be utilized for any given purpose.

The following examples are given as illustrative of the process of the present invention specifically with the use of different compounds as solvent A. It is to be understood that these examples are in no way meant to limit the scope of the present invention.

#### Example I

To a gel consisting of 20 parts aluminum naphthenate and 80 parts of purified light petroleum is added while stirring at a temperature of 25° C., 5 parts of pentapropylene-glycoldodecylether. This causes a sudden change from gelatinous condition to a thinly liquid, easily pourable solution.

#### Example II

The great viscosity-lowering effect of laurylpentapropylene glycol is illustrated by mixing with mineral oils containing various naphthenic acid salts. This is shown on the following table. The various naphthenic acid salts in the amounts given in the table were each stirred with 100 parts by weight of a mineral oil (specific gravity at 20° C.—0.882; viscosity index—89; coking number according to Conradson—0.11; and portion insoluble in gasoline—0) at a temperature of 100-110° C. until a homogeneous mixture was obtained and the viscosities of these mixtures were measured at 80° C. or 50° C. as indicated. The same solutions were then mixed with the given parts by weight of laurylpentapropylene-glycolether and the viscosity of these solutions were measured at 80° C. or 50° C., as indicated.

| Naphthenate                           | Parts by Weight | Parts by Weight laurylpentapropylene glycol ether | Viscosity     |        |
|---------------------------------------|-----------------|---------------------------------------------------|---------------|--------|
|                                       |                 |                                                   | temp. in ° C. | cst.   |
| Aluminum naphthenate.....             | 1               | 0.4                                               | 80            | 27.59  |
| Do.....                               | 1               | 0.4                                               | 80            | 19.80  |
| Aluminum and Calcium naphthenate..... | 5+5             | 4                                                 | 80            | 49.99  |
| Do.....                               | 5+5             | 4                                                 | 80            | 30.00  |
| Zinc naphthenate.....                 | 30              | 4                                                 | 80            | 72.76  |
| Do.....                               | 30              | 4                                                 | 80            | 37.04  |
| Iron naphthenate.....                 | 30              | 4                                                 | 50            | 119.02 |
| Do.....                               | 30              | 4                                                 | 50            | 108.20 |
| Lead naphthenate.....                 | 30              | 4                                                 | 50            | 85.20  |
| Do.....                               | 30              | 4                                                 | 50            | 78     |

#### Example III

The viscosity lowering effect of polyalkylene glycol derivatives is also achieved on naphthenate solutions which already have a low viscosity. A solution of 30

parts by weight calcium naphthenate in 100 parts by weight of a hydrocarbon of diesel oil character has at 80° C. a viscosity of 3.02 cst. The addition of 8 parts by weight of methylheptaethyleneglycolnaphthenicacid-ester to 100 parts by weight of the solution causes a 5 lowering of the viscosity at 80° C. to 2.74 cst.

*Example IV*

Mineral oil having the viscosity at 80° C. of 18.70 cst. has the viscosity thereof increased by dissolving 10% 10 by weight of potassium naphthenate therein, to a value at 80° C. of 29.5 cst. An addition of 20% decylpentapropyleneglycoether causes a reduction of the viscosity at 80° C. to 21.26 cst. A methyl ether or the benzoate of the polyalkyleneglycoether mentioned above will 15 have the same effect.

*Example V*

100 parts by weight of Tetralin and 20 parts by weight of barium naphthenate result in a solution having an 20 average viscosity at 80° C. of 15.5 cst. The addition to 100 parts by weight of this solution of 10 parts by weight of laurylpentaethyleneglycoether results in a lowering of the viscosity at 80° C. to 1.76 cst.

*Example VI*

Neutral barium naphthenate from distilled naphthenic acid having an acid number of 180 and is in the form of a brittle resin at room temperature, in gummy state at a temperature of 100° C. and has a drop-forming temperature of more than 230° C. This substance is extremely difficult to dissolve in mineral oil and after cooling a solution of the same in mineral oil a heavy gelatin-like mass is formed.

A fatty alcohol having a hydroxyl number of 6.8 obtained by high pressure hydrogenation of paraffin-oxidized fatty acid forms with 5 moles of ethylene oxide using an alkali as catalyst of the oxethylation a waxy mass at room temperature having a drop-forming point of 38° C.

By mixing 40 parts of the brittle barium naphthenate with 15 parts of the polyglycol ether at 100° C. while stirring, the gummy-like structure of the substance is changed and upon cooling a thread-drawing syrup is obtained which is easily soluble in hydrocarbons without the formation of any undissolved residues.

In addition to the above described polyalkylene glycol derivatives which serve as solvent A, it is desirable to add a high boiling point ether (solvent B) to the mixture to increase the dissolving ability of the hydrocarbon and to further lower the viscosity of the formed solution. The high boiling point ethers which serve as solvent B are monoethers having the general formula R'-O-R" wherein at least one of the radicals R' and R" consists of 6 or more carbon atoms. The radicals R' and R" may be aliphatic, aromatic, or alicyclic and may be derived from mono- or polyhydric alcohols. However, in the event that the radical is derived from a polyhydric alcohol, the polyhydric alcohol must not have any ether linkages in the molecule except the single ether linkage with the other radical, namely R' or R". In other words the high boiling point ether must have only one ether linkage so that the same is free of polyalkylene glycol groups. It is this lack of polyalkylene glycol groups of solvent B which is the distinguishing feature between solvent B and solvent A. It is advantageous that the high boiling point monoether serving as solvent B be liquid at room temperature.

It has been found according to the present invention that the high boiling point ethers of solvent B seem to 70 serve as intermediate solvent not only for the naphthenic acid salts but also for the solvent A in the hydrocarbon solvent.

The following are examples of high boiling point mono-ethers according to the present invention. It is 75

to be understood that these are illustrative only of the many compounds which may be used as solvent B and the scope of the present invention is in no way limited to the specific compounds mentioned:

Di-n-hexylether, di-n-octylether, di-n-nonyl-ether, di-2-ethylhexylether, lauryl-2-ethylhexylether, octadecen-9-yl-1-isobutylether, dodecylphenylether, laurylcyclohexylether, octyl-B-tetraloether, nonyl-4-methyl-cyclohexylether, 4- octylphenyl- 2-ethylhexylether, etc. Benzyl ethers or alkyl substituted benzyl ethers of the above named or other aliphatic or alicyclic alcohols may also be used, i.e. nonylbenzylether, octadecenyl-4-methylbenzylether, di-benzylether, tetrahydronaphthylmethyl-phenyl- or benzylether, tetrahydronaphthylmethyl-2-ethylhexylether, butandiol-(1,3)-monoocystylether, butandiol-(1,4)-dibenzylether, and butandiol-(1,4)-isobutyl-dodecylether.

As may be seen from the above, at least one of the radicals R' and R" must be of at least 6 carbon atoms. There is no actual limit to the number of carbon atoms of either or both of the radicals though as a practical matter, radicals having less than 24 carbon atoms are preferred.

25 Ethers from paraffin fatty alcohols or their first runnings upon distillation as well as the oxo- or naphthene alcohols are particularly suitable, i.e. paraffin fatty alkyl-cyclohexylether, the first running upon distillation of dodecylalkylether, etc. The term "first running" is to be understood as meaning the first distillate of a mixture of alcohols obtained from high pressure hydrogenation of paraffin fatty acids whereby the alcohols of the mixture have a chain length of 6-9 carbon atoms.

30 The naphthenic acids are those obtained by raffination of mineral oils, which by high pressure reduction or by the process of Bouveault-Blanc may be transformed into the corresponding naphthene alcohol which may be easily reacted to form the ether. As examples of ethers which may be produced by the above described methods are, dinaphthenylether, and naphthenyl-benzyl- and -2- ethylhexylether.

35 It is possible to use either single ether or mixtures of two or more ethers or ether solutions or mixtures of ethers in hydrocarbons and hydrocarbon oils.

40 The application of a high boiling point monoether, namely solvent B increases the dissolvability of the naphthenic acid salts in the hydrocarbon or hydrocarbon oil. Whereas a mixture of a naphthenate with a solvent A at room temperature may form a waxy mass, the addition of 45 20% of a solvent B or mixture of ethers constituting the solvent B, transforms the waxy mass into a clear solution. The resulting clear solution may be easily diluted with a liquid hydrocarbon.

45 Besides acting as intermediate solvent, the ethers of solvent B also have the effect of lowering the viscosity of 50 solutions of naphthenic acid salts, solvent A and hydrocarbon.

55 The amount of high boiling point monoether which may be utilized varies within very wide limits i.e. from 60 very small amounts to twice the amount of a naphthenate and solvent A, or even more. The amount of solvent B is not only dependent upon the type and amount of naphthenic acid salt or mixture of naphthenic acid salt with solvent A, but also upon the degree of solubility which is desired and the desired miscibility of the naphthenic acid salt in the liquid hydrocarbon and also upon the desired viscosity of the final solution.

65 The production of naphthenic acid salt solutions in liquid hydrocarbons in the presence of at least one solvent A and at least one solvent B may be accomplished in many ways. For example the naphthenate may first be dissolved in the solvent B and the solvent A solution added thereto; and then adding the hydrocarbon oil thereto. It is also possible to first form a solution or paste of the naphthenic acid salt and the solvent A and

to then add to this mixture a solvent B; and finally to add a liquid hydrocarbon to the combined mixture. It is also possible to first form a solution of the liquid hydrocarbon, solvent A and solvent B and to dissolve the naphthenic acid salt in the thus formed solution. It is still further possible to dissolve the naphthenic acid salt in solvent B and to dissolve solvent A in solvent B and then mix the two solutions to form a single solution thereof which may be easily mixed with a liquid hydrocarbon.

The following examples are given as illustrative of the use of a solvent B in addition to a solvent A for the production of solutions of naphthenic acid salt.

#### Example VII

This example illustrates how the addition of a solvent B forms a clear solution of a naphthenate in a solvent A. Various naphthenates of the cations indicated in the following table were mixed with the polyalkylene glycol derivative indicated in the table in the proportion of 10:1 at a temperature of 40-80° C. Upon cooling a waxy mass was obtained. This mixture was then mixed in proportion of 1:1 with a solvent B ether indicated in the table. The addition of the ether to the mixture resulted in every case in the formation of a thin liquid solution which could be easily dissolved in a hydrocarbon.

| Cation           | Polyalkyleneglycol-derivative              | Ether                             |
|------------------|--------------------------------------------|-----------------------------------|
| potassium        | naphthenic acid-hepta-alkyleneglycolester. | ethylhexyl-benzyl ether.          |
| tin**            | dodecyl-pentaethylene-glycolmethylether.   | lauryl-n-butylether.              |
| lead             | benzylpentapropylene-glycolbenzoate.       | diocetyl-ether.                   |
| iron***          | p-octylphenyltetrapropylene-glycolether.   | dibenzylether.                    |
| aluminum/calcium | stearyl-hexaethylene-glycolbenzoate.       | tetradecylmethyl cyclohexylether. |

#### Example VIII

Neutral aluminum naphthenate is very poorly soluble in a hydrocarbon such as petroleum or mineral oil. By stirring for a long time at a raised temperature of 100° C. a solution is formed which is in the form of a tough gel which upon cooling becomes non-homogeneous, a portion of the petroleum or mineral oil separating therefrom. The viscosity which is very difficult to measure with the above solution may be judged to be approximately 6000 cst. at 80° C. This gel is unsuitable for all technical purposes wherein a solution of aluminum naphthenate is desired. An addition of 4% laurylpentapropylene-glycolether lowers the viscosity of the aluminum naphthenate solution in the hydrocarbon from a value above 6000 to about 160 cst.

It is further preferable to first dissolve the aluminum naphthenate in a high boiling ether of solvent B. By dissolving 10 parts by weight aluminum naphthenate in 100 parts dodecyl-2-ethylhexylether a solution having a viscosity of 1890 cst. at 80° C. is obtained. The viscosity is further lowered by the addition of 4% laurylpentapropylene glycol to about 99 cst. This solution is miscible in all proportions with hydrocarbons and results in the formation of thin fluid solutions.

#### Example IX

A solution of 50% calcium naphthenate in dodecyl-octylether has a viscosity of 18.60 cst. at a temperature of 80° C. and upon the addition of 10% dodecylpentapentaethylene-glycolether the viscosity is lowered to 11.4 cst.

#### Example X

The lowering of the viscosity of the mixture of 60 parts barium naphthenate and 30 parts laurylpenta-

8  
ethyleneglycoether by the addition of varying amounts of laurylethylhexylether is shown in the following table:

| Percent by weight of laurylethylhexylether added | Viscosity of the mixture at 80° C. in cst. |
|--------------------------------------------------|--------------------------------------------|
| 0                                                | 122.0                                      |
| 20                                               | 38.1                                       |
| 40                                               | 18.5                                       |
| 60                                               | 12.5                                       |
| 80                                               | 9.2                                        |
| 100                                              | 7.7                                        |

#### Example XI

15 A 50% solution of barium naphthenate in a hydrocarbon such as of the spindle oil type can be formed only with very great difficulties and is unsuitable for all technical purposes. A solution of equal concentration of the 20 naphthenate in laurylethylhexylether is comparatively easy to produce and has a viscosity of 2335 cst. at 80° C. By the addition to the above of a polyalkylene-glycol derivative the viscosity is lowered. The lowering of the viscosity is dependent to some extent on the degree of 25 polymerization of the polyalkylene-glycol derivative. This is illustrated as follows:

|                                        | Viscosity at 80° C., cst. |
|----------------------------------------|---------------------------|
| 20% lauryl-triethyleneglycoether       | 11.80                     |
| 20% lauryl-pentaethylene-glycoether    | 11.94                     |
| 30 20% lauryl-heptaethylene-glycoether | 13.38                     |

If the viscosity lowering substance laurylhexaethyleneglycoether is further etherified with ethylhexanol to laurylhexaglycoethylhexylether, the viscosity lowering remains within the same limits and the 20% addition will result in a solution having a viscosity of 13.64 cst.

Any of the above solutions may be easily mixed with liquid hydrocarbons.

#### Example XII

40 This example illustrates the viscosity lowering effect of 45 various polyalkylene-glycol derivative on a 50% barium naphthenate solution in laurylethylhexylether. The original solution has the viscosity of 3255 at 80° C. The polyalkylene-glycol derivatives indicated were added in an amount of 20% and the resulting viscosity at 80° C. was as indicated:

|                                       | Cst. |
|---------------------------------------|------|
| Benzylpentapropylene-glycoether       | 10.4 |
| Octylphenoloctapropylene-glycoether   | 15.5 |
| Stearicacid heptapropylene-glycoether | 14.0 |

55 The addition of the naphthenic acid salts to a motor oil by means of a solvent A with or without a solvent B improves the activity of the motor oil even at low temperatures of i.e. 40-50° C. Likewise the addition to a lubricating oil also increases the action of the lubricating oil. The amount to be added to the motor oil or lubricating oil depends upon the sulfur content of the oil, and other properties and characteristics thereof. The amount may vary within rather wide limits, though generally amounts between 0.5-10% by weight of the naphthenate and solvent A with or without solvent B is suitable.

60 The following examples are given to illustrate the use of the present invention on the formation of motor and lubricating oils of improved properties.

#### Example XIII

A mixture is formed of:

|                                                                                                                                                                       |
|-----------------------------------------------------------------------------------------------------------------------------------------------------------------------|
| 70 40 parts laurylethylhexylether                                                                                                                                     |
| 15 parts of a pentaethylene-glycoether of a fatty alcohol obtained by high pressure hydrogenation of a paraffin-oxygenated fatty acid having a hydroxyl number of 6.6 |
| 40 parts barium naphthenate and                                                                                                                                       |
| 75 5 parts p-ethylhexylphenol                                                                                                                                         |

5 parts of this mixture is mixed with 95 parts of a basic paraffin oil having the following properties:

Specific gravity at 30° C. 0.885  
Flash point ° C. 225  
Viscosity at 50° C. cst. 65.8

In a diesel motor measuring device the above motor oil mixture is found to have the following characteristics:

Oil temperature 100° C.; and testing time 120 hours with a full load. The oil utilized was Middle East diesel oil having the sulfur content of 1%.

Upon ending the test run all the piston rings were freely movable and showed no slime or carbon deposits. The outside as well as the inside of the piston rings had a predominantly metallic appearance.

Tests as to the lubricating properties of the used oil on an Almen-Wieland machine gave a u-value between 0.2-0.1 with a possible load of 28 plates (1400 kg.).

*Example XIV*

The following mixture was tested:

65 parts lauryl ethylhexylether  
15 parts laurylpentapropylene glycol ether  
36 parts barium naphthenate  
5 parts ethylhexylphenol

To a basic paraffin oil as in Example XIII was added 10% by weight of the above mixture and the resulting mixture was tested as a motor oil. The driving distance was 6000 kilometers without any oil change, the used oil only being replaced.

Upon ending the test drive the piston rings and the oil scraper rings were freely movable and no carbon or slime deposits were found in the piston grooves. The piston surface and cylinder walls had a true metallic appearance.

Tests as to the lubricating properties of the used oil in the Almen-Wieland machine showed a u-value between 0.1 and 0.2 and with a possible load of 20 plates (1000 kg.).

*Example XV*

In a two stroke diesel engine the following mixture as an addition of 10% to the above lubricating oil was tested:

20 parts barium naphthenate  
15 parts calcium naphthenate  
15 parts napthenealcohol-hexaethyleneglycolether  
45 parts diethyl ether  
5 parts di-tertiary-butyl-p-cresol

After a ten hour test run at 4500 revolutions per minute and at a water temperature of 95° C. the piston rings were freely movable and the surfaces thereof were of metallic appearance both on the inner and on the outer surface.

Without further analysis, the foregoing will so fully reveal the gist of the present invention that others can by applying current knowledge readily adapt it for various applications without omitting features that, from the standpoint of prior art, fairly constitute essential characteristics of the generic or specific aspects of this invention and, therefore, such adaptations should and are intended to be comprehended within the meaning and range of equivalence of the following claims.

What is claimed as new and desired to be secured by Letters Patent is:

1. A process of forming liquid hydrocarbon solutions of naphthenic acid salts, comprising the steps of mixing a naphthenic acid salt with a liquid hydrocarbon at a temperature of 90-150° C.; and adding at said temperature to the thus formed mixture at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 6 carbon atoms in an amount sufficient to form a solution of said naphthenic acid salt, said liquid hydrocarbon and said substance.

2. A process of forming liquid hydrocarbon solutions of naphthenic acid salts, comprising the steps of mixing at a temperature of 90-150° C. a liquid hydrocarbon with at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 6 carbon atoms; and adding at said temperature to the thus formed mixture a naphthenic acid salt, said substance being present in an amount sufficient to form a solution of said liquid hydrocarbon, said naphthenic acid salt and said substance.

3. A process of forming liquid hydrocarbon solutions of naphthenic acid salts, comprising the steps of mixing at a temperature of 90-150° C. a naphthenic acid salt with at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 6 carbon atoms;

45 and adding at room temperature to the thus formed mixture a liquid hydrocarbon, said substance being present in an amount sufficient to form a solution of said liquid hydrocarbon, said naphthenic acid salt and said substance.

4. A process of forming liquid hydrocarbon solutions of naphthenic acid salts, comprising the steps of dissolving a naphthenic acid salt in at least one warm substance having the general formula:



55 wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic, and acyl radicals and the other of said groups X and Y is selected from the class consisting of alkyl, aryl, aralkyl, alkaryl, alicyclic and acyl radicals having at least 6 carbon atoms;

60 adding to the thus formed solution at least one high boiling point monoether having the general formula:



70 wherein R' and R'' are selected from the group consisting of alkyl, aryl, aralkyl, alkaryl, and alicyclic radicals and at least one of the groups R' and R'' contains at least 6 carbon atoms, thereby forming a combined solution thereof; and adding a liquid hydrocarbon to the thus formed combined solution said substance and said high boiling point monoether being present in an amount sufficient to form a solution of said liquid hydrocarbon,

said naphthenic acid salt, said substance and said high boiling point monoether.

5. A process of forming liquid hydrocarbon and hydrocarbon oil solutions of naphthenic acid salts, comprising the steps of dissolving a naphthenic acid salt in at least one high boiling point monoether having the general formula:



wherein R' and R'' are selected from the group consisting alkyl, aryl, aralkyl, alkaryl, and alicyclic radicals and at least one of the groups R' and R'' contains at least 6 carbon atoms; adding to the thus formed solution at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 6 carbon atoms, said substance being in an amount of 1% to equal the weight of said naphthenic acid salt, and said high boiling point monoether being in an amount up to two-times the amount of said naphthenic acid salt plus said substance, thereby forming a combined solution, of said naphthenic acid salt, said substance and said high boiling point monoether and mixing the thus-formed combined solution with a liquid hydrocarbon, thereby forming a hydrocarbon naphthenic acid salt solution the proportions of which may be varied in all proportions while still retaining a true solution.

6. As a new product, a hydrocarbon motor oil containing in solution between 0.5-10% by weight of a naphthenic acid salt and at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 6 carbon atoms, said substance being present in an amount from 1% to equal the weight of said naphthenic acid salt.

7. As a new product, a hydrocarbon lubricating oil containing in solution between 0.5-10% by weight of a naphthenic acid salt and at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 6 carbon atoms, said substance being present in an amount from 1% to equal the weight of said naphthenic acid salt.

8. As a new product, a hydrocarbon motor oil containing in solution between 0.5-10% by weight of a naphthenic acid salt, at least one substance having the general formula:



wherein R is an alkylene radical having a minimum of 2 and a maximum of 3 carbon atoms, n is a whole number

between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 6 carbon atoms, said substance being present in an amount from 1% to equal the weight of said naphthenic acid salt and at least one high boiling point monoether having the general formula:



wherein R' and R'' are selected from the group consisting of alkyl, aryl, aralkyl, alkaryl, and alicyclic radicals and at least one of the groups R' and R'' contains at least 6 carbon atoms, said high boiling point monoether being present in an amount of 10% to up to two times the weight of said naphthenic acid salt plus said substance.

9. As a new product, a hydrocarbon lubricating oil containing in solution between 0.5-10% by weight of a naphthenic acid salt, at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 6 carbon atoms, said substance being present in an amount from 1% to equal the weight of said naphthenic acid salt and at least one high boiling point monoether having the general formula:



wherein R' and R'' are selected from the group consisting of alkyl, aryl, aralkyl, alkaryl, and alicyclic radicals and at least one of the groups R' and R'' contains at least 6 carbon atoms, said high boiling point monoether being present in an amount of 10% to up to two times the weight of said naphthenic acid salt plus said substance.

10. As a new product, a hydrocarbon motor oil containing in solution between 0.5-10% by weight of barium naphthenate and at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 6 carbon atoms, said substance being present in an amount from 1% to equal the weight of said barium naphthenate.

11. A liquid hydrocarbon solution consisting essentially of a liquid hydrocarbon; a naphthenic acid salt; and at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 6 carbon atoms in an amount sufficient to form a solution of said naph-

thenic acid salt, said liquid hydrocarbon and said substance.

12. A liquid hydrocarbon solution consisting essentially of a liquid hydrocarbon; a naphthenic acid salt; and at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 8 carbon atoms in an amount sufficient to form a solution of said naphthenic acid salt, said liquid hydrocarbon and said substance.

13. A liquid hydrocarbon solution consisting essentially of a liquid hydrocarbon; a naphthenic acid salt; and at least one substance having the general formula;



wherein R is an alkylene radical having a minimum of 2 and a maximum of 3 carbon atoms, n is a whole number between 2 and 7, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 8 carbon atoms in an amount sufficient to form a solution of said naphthenic acid salt, said liquid hydrocarbon and said substance.

14. A liquid hydrocarbon solution consisting essentially of a liquid hydrocarbon; a naphthenic acid salt; and at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 12 carbon atoms in an amount sufficient to form a solution of said naphthenic acid salt, said liquid hydrocarbon and said substance.

15. A liquid hydrocarbon solution consisting essentially of a liquid hydrocarbon; a naphthenic acid salt; and at least one monoether of a radical selected from the group consisting of alkyl, aryl, aralkyl, alkaryl, and alicyclic radicals having at least 6 carbon atoms and a polyalkylene glycol having a minimum of 2 and a maximum of 3 carbon atoms in the alkylene group and having a maximum of 21 alkylene groups in an amount sufficient to form a solution of said liquid hydrocarbon, said naphthenic acid salt and said monoether.

16. A liquid hydrocarbon solution consisting essentially of a liquid hydrocarbon; a naphthenic acid salt; and at least one diether of a polyalkylene glycol having a minimum of 2 and a maximum of 3 carbon atoms in the alkylene group and having a maximum of 21 alkylene groups, said polyalkylene glycol being etherified at both ends of the polyalkylene glycol chain with a radical selected from the group consisting of alkyl, aryl, aralkyl, alkaryl, and alicyclic radicals at least one of which has at least 6 carbon atoms in an amount sufficient to form a solution of said liquid hydrocarbon, said naphthenic acid salt and said diether.

17. A liquid hydrocarbon solution consisting essentially of a liquid hydrocarbon; a naphthenic acid salt; and at least one monoester of an acyl radical selected from the group consisting of alkyl, aryl, aralkyl, alkaryl, and alicyclic radicals having at least 6 carbon atoms

and a polyalkylene glycol having a minimum of 2 and a maximum of 3 carbon atoms in the alkylene group and having a maximum of 21 alkylene groups in an amount sufficient to form a solution of said liquid hydrocarbon, said naphthenic acid salt and said monoester.

5 18. A liquid hydrocarbon solution consisting essentially of a liquid hydrocarbon; a naphthenic acid salt; and at least one diester of a polyalkylene glycol having a minimum of 2 and a maximum of 3 carbon atoms in the alkylene group and having a maximum of 21 alkylene groups, said polyalkylene glycol being esterified at both ends of the polyalkylene glycol chain with acyl radicals at least one of which has at least 6 carbon atoms in an amount sufficient to form a solution of said liquid hydrocarbon, said naphthenic acid salt and said diether.

10 19. A liquid hydrocarbon solution consisting essentially of a liquid hydrocarbon; a naphthenic acid salt; and at least one derivative of a polyalkylene glycol having a minimum of 2 and a maximum of 3 carbon atoms in the alkylene group and having a maximum of 21 alkylene groups, said polyalkylene glycol being etherified at one end of the polyalkylene glycol chain with a radical selected from the group consisting of alkyl, aryl, aralkyl, alkaryl, and alicyclic radicals and being esterified at the other end of said polyalkylene glycol chain with an acyl radical, at least one of said acyl, aryl, aralkyl, alkaryl, alicyclic radicals having at least 6 carbon atoms in an amount sufficient to form a solution of said liquid hydrocarbon, said naphthenic acid salt and said derivative.

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635

carbon atoms said substance and said high boiling point monoether being present in an amount sufficient to form a solution of said liquid hydrocarbon, said naphthenic acid salt, said substance and said high boiling point monoether.

23. A liquid hydrocarbon solution consisting essentially of a liquid hydrocarbon; a naphthenic acid salt; at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 6 carbon atoms in an amount of 1% to equal the weight of said naphthenic acid salt; and at least one high boiling point monoether having the general formula:



wherein R' and R'' are selected from the group consisting of alkyl, aryl, aralkyl, alkaryl, and alicyclic radicals and at least one of the groups R' and R'' contains at least 6 carbon atoms in an amount of 10% to up to two times the amount of said naphthenic acid salt plus said substance.

24. A liquid hydrocarbon solution consisting essentially of a liquid hydrocarbon; a naphthenic acid salt; and at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 6 carbon atoms in an amount of 1% to equal the weight of said naphthenic acid salt; and at least one high boiling point monoether liquid at room temperature and having the general formula:



wherein R' and R'' are selected from the group consisting of alkyl, aryl, aralkyl, alkaryl, and alicyclic radicals and at least one of the groups R' and R'' contains at least 6 carbon atoms and wherein both alkyl groups R' and R'' are derived from monohydric alcohols in an amount of 10% to up to two times the amount of said naphthenic acid salt plus said substance

25. A liquid hydrocarbon solution consisting essentially

ly of a liquid hydrocarbon; a naphthenic acid salt; and at least one substance having the general formula:



wherein R is an alkylene radical having a minimum of 2 and a maximum of 3 carbon atoms, n is a whole number between 1 and 20, and wherein one of the groups X and Y is selected from the class consisting of hydrogen, alkyl, aryl, aralkyl, alkaryl, alicyclic and acyl radicals and the other of said groups X and Y is selected from the class consisting of alkyl, aryl, aralkyl, alkaryl, alicyclic and acyl radicals having at least 6 carbon atoms in an amount of 1% to equal the weight of said naphthenic acid salt; and at least one high boiling point monoether liquid at room temperature and having the general formula:



wherein R' and R'' are selected from the group consisting of alkyl, aryl, aralkyl, alkaryl, and alicyclic radicals and at least one of the groups R' and R'' contains at least 6 carbon atoms and wherein at least one of the alkyl groups R' and R'' is derived from monohydric alcohols in an amount of 10% to up to two times the amount of said naphthenic acid salt plus said substance.

26. A liquid hydrocarbon solution consisting essentially of a liquid hydrocarbon; a naphthenic acid salt; and at least one monoether of a polyalkylene glycol having a minimum of 2 and a maximum of 3 carbon atoms in the alkylene group and having 5 alkylene groups, said polyalkylene glycol being etherified at one end of the polyalkylene glycol chain by an alkyl radical of 12 carbon atoms in an amount of 1% to equal the weight of said naphthenic acid salt, and with dodecyloctyl ether in an amount of 10% to up to two times the amount of said naphthenic acid salt plus said monoether.

27. A liquid hydrocarbon solution consisting essentially of a liquid hydrocarbon; a naphthenic acid salt; and at least one monoether of a polyalkylene glycol having a minimum of 2 and a maximum of 3 carbon atoms in the alkylene group and having 5 alkylene groups, said polyalkylene glycol being etherified at one end of the polyalkylene glycol chain by an alkyl radical of 12 carbon atoms in an amount of 1% to equal the weight of said naphthenic acid salt, and with dodecyl-2-ethylhexyl ether in an amount of 10% to up to two times the amount of said naphthenic acid salt plus said monoether.

#### References Cited in the file of this patent

#### UNITED STATES PATENTS

|    |           |          |               |
|----|-----------|----------|---------------|
| 50 | 1,739,686 | Merrill  | Dec. 17, 1929 |
|    | 2,122,940 | Hodson   | July 5, 1938  |
|    | 2,227,149 | Murphree | Dec. 31, 1940 |

#### OTHER REFERENCES

55 Synthetic Organic Chemicals—pub. of Carbide and Carbon Corp., N. Y., Oct. 15, 1940, page 28.